

## 1

2,910,437

## STABILIZATION OF LUBRICANTS

Ted Symon, Hinsdale, Ill., assignor, by mesne assignments, to Universal Oil Products Company, Des Plaines, Ill., a corporation of Delaware

No Drawing. Application March 9, 1956  
Serial No. 570,420

4 Claims. (Cl. 252—32)

The invention is particularly applicable to the stabilization of greases, either of synthetic or petroleum origin. The synthetic greases generally are referred to as lithium base grease, sodium base grease, calcium base grease, barium base grease, strontium base grease, aluminum base grease, etc. These greases are solid or semi-solid gels and, in general, are prepared by the addition to mineral or synthetic oils of hydrocarbon-soluble metal soaps or salts of higher fatty acids as, for example, lithium stearate, calcium stearate, aluminum naphthenate, etc. The grease may contain thickening agents such as silica, carbon black, polyacrylates, talc, etc. Another type of grease is prepared from oxidized petroleum wax, to which the saponifiable base is combined with the proper amount of the desired saponifying agent, and the resultant mixture processed to produce a grease. Other types of greases in which the features of the present invention are usable include petroleum grease, whale grease, wool grease, etc., and those made from inedible fats, tallow, butcher's waste, etc.

The present invention also is particularly applicable to the stabilization of lubricating oils, including those of petroleum or synthetic origin. The synthetic lubricants are of varied types including aliphatic esters, polyalkylene oxides, silicones, esters of phosphoric and silicic acids, highly fluorine-substituted hydrocarbons, etc. Of the aliphatic esters, di-(2-ethylhexyl) sebacate is being used on a comparatively large commercial scale. Other aliphatic esters include dialkyl azelates, dialkyl suberates, dialkyl pimelates, dialkyl adipates, dialkyl glutarates, etc. Specific examples of these esters include dihexyl azelate, di-(2-ethylhexyl) azelate, di-3,5,5-trimethylhexyl glutarate, di-3,5,5-trimethylpentyl glutarate, di-(2-ethylhexyl) pimelate, di-(2-ethylhexyl) adipate, triamyl tricarboxylate, pentaerythritol tetracaproate, dipropylene glycol dipelargonate, 1,5-pentanediol-di-(2-ethylhexanoate), etc. The polyalkaline oxides and derivatives include polyisopropylene oxide, polyisopropylene oxide diether, polyisopropylene oxide diester, etc. The silicones include methyl silicone, methylphenyl silicone, etc., and the silicates include, for example, tetraisoctyl silicate, etc. The highly fluorinated hydrocarbons include fluorinated oil, perfluorohydrocarbons, etc.

In a specific embodiment the present invention relates to a method of stabilizing synthetic grease which comprises incorporating therein from about 0.1 to about 5% by weight of 2,4'-diaminodiphenyl ether.

In another embodiment the present invention relates to a method of stabilizing lubricating oil against oxidative deterioration which comprises incorporating therein a stabilizing concentration of a 2,4'-diaminodiphenyl ether.

In one embodiment the present invention comprises a 2,4'-diaminodiphenyl ether. A preferred inhibitor is 2,4'-diaminodiphenyl ether.

In general, the inhibitor will be utilized in a concentration of from about 0.0001% to about 5% by weight of the organic substance, although in some cases higher

## 2

or lower concentrations may be employed. The exact concentration to be used will depend upon the particular organic substance being treated. In most cases concentrations of from about 0.01% to about 3% by weight generally will be employed.

It is understood that the inhibitor may be used along with other additives incorporated in the organic substance. For example, in grease the inhibitor may be used along with higher alcohols, esters, organic amines, polybutene, sulfurized fatty materials, sulfur chlorine compounds, dyes, perfumed materials, fillers, etc. In some cases, it may be of advantage to also include a metal deactivator as, for example, disalicylal diamino propane, ethylene diamine tetra-acetic acid tetrasodium salt, etc., or to include other additives such as tricresyl phosphate, trialkyl phenols including 2,6-di-tert-butyl-4-methylphenol, 2,4-di-methyl-6-tert-butylphenol, alkylated diphenyl amines, phenyl naphthyl amines, dialkyl phenylene diamines, phenothiazine, organic selenium compounds, etc., as well as corrosion inhibitors, extreme pressure additives, viscosity index improvers, etc. When desired, the inhibitor of the present invention may be prepared as a mixture with one or more of these other additives and incorporated in this manner in the organic substance or components thereof.

The inhibitor of the present invention may be incorporated in the organic substance in any suitable manner and at any suitable stage of preparation. For example, in an organic substance which comprises a mixture of several components, as for example, grease, the inhibitor may be added to one or more of the components of the grease prior to compounding and processing thereof or it may be added to the mix at any time, preferably before final processing in order to obtain intimate mixing and dissolving of the inhibitor in the grease.

The following examples are introduced to illustrate further the novelty and utility of the present invention but not with the intention of unduly limiting the same.

*Example I*

2,4'-diaminodiphenyl ether was utilized as an inhibitor in a lithium grease. The grease was prepared by mixing 91% of a Pennsylvania bright stock with 8% of lithium stearate. The mixture was heated at about 450° F. while agitating the same. Subsequently, the grease was cooled while agitating to 320° F. and, at this temperature, 1% of 2,4'-diaminodiphenyl ether was added. Agitation was continued and the mixture was allowed to cool to about 250° F. and the grease then further cooled slowly to room temperature.

The stability of the grease was tested according to a modified Norma Hoffman method, in which a sample of the grease is placed in a bomb in the presence of brass discs acting as an oxidation catalyst and oxygen is charged thereto. The bomb then is heated to 212° F., and the time required for a drop of 5 pounds pressure is taken as the induction period. In this run, a control sample of the grease (not containing this additive) had an induction period of 10.5 hours. On the other hand, a sample of the grease containing 1% by weight of 2,4'-diaminodiphenyl ether had an induction period of 260 hours. Thus, it will be noted that the inhibitor of the present invention was exceptionally effective in improving the stability of the grease.

*Example II*

The grease used in this example was prepared in substantially the same manner as described in Example I except that a Mid-Continent lubricating oil having a S.A.E. viscosity of 30 was used.

This grease had a control (not containing this additive) induction period of 10.5 hours. On the other hand,

a sample of this grease containing 1% by weight of 2,4'-diaminodiphenyl ether had an induction period of 370 hours. Here again, it will be noted that the inhibitor of the present invention was exceptionally effective in improving the stability of the grease.

*Example III*

The grease used in this example was a synthetic grease prepared in substantially the same manner described in Example I, except that 87% of di-2-ethylhexyl sebacate was mixed with 12% lithium stearate. 1% by weight of 2,4'-diaminodiphenyl ether was incorporated in the synthetic grease. A control sample of the grease (not containing this additive) had an induction period of 17 hours. On the other hand, a sample of the grease containing 1% by weight of 2,4'-diamino-diphenyl ether did not undergo a pressure drop of one pound per square inch until after 318 hours exposure.

From the above data, it will be noted that this inhibitor was very effective in improving the stability of the synthetic grease.

I claim as my invention:

1. A method of stabilizing a lubricant normally subject to oxidative deterioration which comprises incorporating

therein a stabilizing concentration of 2,4'-diaminodiphenyl ether.

2. A lubricant normally subject to oxidative deterioration containing, as an inhibitor against said deterioration, a stabilizing concentration of 2,4'-diaminodiphenyl ether.

3. Grease normally tending to undergo oxidative deterioration containing, as an inhibitor against said deterioration, a stabilizing concentration of 2,4'-diaminodiphenyl ether.

4. Lubricating oil tending to undergo oxidative deterioration containing as an inhibitor against said deterioration, a stabilizing concentration of 2,4'-diaminodiphenyl ether.

References Cited in the file of this patent

UNITED STATES PATENTS

|           |                 |                |
|-----------|-----------------|----------------|
| 2,048,362 | Stoesser et al. | July 21, 1936  |
| 2,269,265 | Hamilton et al. | Jan. 6, 1942   |
| 2,290,860 | Burk et al.     | July 28, 1942  |
| 2,350,746 | Fuller          | June 6, 1944   |
| 2,367,264 | Burk et al.     | Jan. 16, 1945  |
| 2,440,530 | Yates           | Apr. 27, 1948  |
| 2,523,100 | Eby             | Sept. 19, 1950 |